

## UNITED STATES PATENT OFFICE

CARL SATTLER, OF KREFELD, GERMANY, ASSIGNOR TO THE FIRM DEUTSCHE EDELSTAHLWERKE AKTIENGESELLSCHAFT, OF KREFELD, GERMANY

## PERMANENT MAGNET

No Drawing. Application filed February 19, 1930, Serial No. 429,832, and in Germany March 8, 1929.

Up to now magnetic chromium and magnetic tungsten steels have been principally used for the production of permanent magnets. Since about ten years the magnetic cobalt steel has been added to satisfy greater demands. The latter, as a rule, being produced with a cobalt content of over 3%. In order to satisfy particularly great demands the cobalt content is being raised to 10, 15, 20 and 35%. Cobalt is still very expensive and the use of magnetic cobalt steel is still a very limited one. Since years the electro-technical industry is in search of a magnetic steel for use on a large scale which is not considerably more expensive than tungsten steel, yet surpasses the latter as regards the magnetic power. The present invention provides such a magnetic steel. This new magnetic steel is based upon the combination of steel alloys which, in addition to 1.3 to 6.5% of chromium as the basic alloying constituent, contain tungsten or molybdenum or vanadium or copper or cobalt or manganese or a mixture of two or more or all of these alloying metals. The presence of at least two of these alloying metals increases the coercive force of the magnetic steel. In order to prove this two alloys had been made one of which contained 0.61% C, 5.5% W, and 2.13% Cr in addition to 0.35% Mn. As a counter-proof a tungsten steel had been produced with 0.60% C, 5.8% W, and 0.33% Mn. In the former case the remanence was 10500 and the coercive force 68 gauss, whereas in the case of the tungsten steel test piece the remanence was 12000, the coercive force, however, only 60 gauss.

In carrying out a number of other tests in which in addition to chromium, tungsten or molybdenum or both were present, it has been found that the addition of one or both these metals increases the coercive force considerably as compared with the corresponding steel containing only chromium. If in addition to chromium and manganese tungsten alone is added, it will be necessary, with a chromium content of only 1.3 to about 1.9%, to add at least 0.8% of tungsten for the purpose of obtaining the highest mag-

netic efficiency. With a chromium content of 4.5% and more a smaller amount of tungsten may be added.

If in addition to chromium and manganese molybdenum alone is added, the molybdenum content has to amount to at least 0.8% with an upper limit of 1.5% in order to obtain a maximum magnetic efficiency. With these percentages, however, the remanence will be considerably lowered. Therefore, in order to secure the beneficial action of the molybdenum all the same, it will prove of advantage to use smaller amounts of molybdenum—about 0.3 to 0.6%—adding thereto tungsten or cobalt or copper either separately or in suitable combination. By properly regulating the proportions of tungsten and molybdenum relatively to the chromium content, one is enabled to produce, with a suitable carbon content which has to range from 0.65 to 1.25%, magnetic steels having a particularly high degree of remanence together with a perfectly satisfactory coercive force or, alternately, steels having a particularly high coercive force together with a satisfactory degree of remanence. If the coercive force rises above 80 gauss up to 100 gauss, the remanence will drop below 10000 gauss. Yet by suitably proportioning the content of carbon, chromium, tungsten and molybdenum, it becomes possible to raise the remanence to above 10000 gauss and the coercive force up to 80 gauss, i. e. to secure a magnetic power factor of  $Br. Hc. 10^{-8} \geq 800$  (Gumlich's numbers), in contradistinction to the best tungsten steels which scarcely give better results than  $Br. Hc. 10^{-8} = 760$ . An increase in the magnetic power factor is more easily brought about by the addition of cobalt in quantities already as small as up to 3%. A magnetic steel with about 3% of chromium and 2% of cobalt is, by way of example, not considerably more expensive than a 6% tungsten steel, yet by far its superior as regards the magnetic properties.

On the other hand, the manufacturing costs of a magnetic steel containing about 2% of chromium and 1% of tungsten or of a magnetic steel containing about 2% of chromium, 0.4% of molybdenum and 0.6% of tungsten

are less by more than 20% than those of a 6% tungsten steel, yet its magnetic properties are equal to those of the best tungsten steel. Similar conditions will prevail if with a chromium content of 1.3 to 6.5% copper in amounts of about 0.5% is added in the place of tungsten or molybdenum. Also copper or vanadium or these metals together with tungsten and molybdenum and with cobalt may be added at the same time. All these metals will considerably increase the coercive force of a magnetic steel having a chromium content as alloying basis. Thus a test piece containing 4.75% Cr. and 1.57% Mo. had a coercive force of 79 gauss.

Having thus described my invention what I claim as new and desire to secure by Letters Patent is:

1. Permanent magnets characterized by the fact that they are produced from steel alloys which contain 0.65% to 1.25% of carbon and about 0.25 to 1% of manganese and in addition to 1.3% to 6.5% of chromium one of the following alloying constituents: tungsten (0.5 to 3%), molybdenum (0.5% to 1.5%), copper (0.5 to 1%) and cobalt (0.5 to 3%).

2. Permanent magnets characterized by the fact that they are produced from steel alloys which contain 0.65 to 1.25% of carbon and about 0.25 to 1% of manganese and in addition to 1.3% to 6.5% of chromium several of the following alloying constituents: tungsten (up to 3%), molybdenum (up to 1.5%), copper (up to 1%) and cobalt (up to 3%), the total percentage of said alloying constituents amounting to a minimum limit of 0.6 and a maximum limit of 7%.

3. Permanent magnets according to claim 1 in which the alloying metals tungsten, molybdenum, copper and cobalt are replaced at least partially by vanadium.

4. Permanent magnets according to claim 2 in which the alloying metals tungsten, molybdenum, copper and cobalt are replaced at least partially by vanadium.

CARL SATTLER.